

## UNITED STATES PATENT OFFICE

2,303,398

## ALKALINE DETERGENT

Charles Schwartz, Pittsburgh, Pa., assignor to  
Hall Laboratories, Inc., Pittsburgh, Pa., a corporation of Pennsylvania

No Drawing. Application May 1, 1939,  
Serial No. 271,177

9 Claims. (Cl. 252—135)

This invention relates generally to alkaline preparations, for example alkaline detergents for cleaning soft metals and more particularly to such detergents containing an inhibiting agent for preventing the alkaline corrosion of the metal.

It is a well known fact that many highly alkaline detergents while performing excellently as cleaners can not be used for the cleaning of soft metals such as aluminum and tin, since the alkalies corrode and dissolve the metals quite readily.

Many efforts have been made to utilize the excellent detergent properties of highly alkaline mixtures and at the same time to prevent, in so far as possible, the attack upon soft metals. Thus the use of certain silicates has been successful in decreasing to a considerable extent the corrosion of aluminum in alkaline solutions. It is necessary, however, to be very careful in the choice of silicate used and in the concentration of the solution in order to avoid very serious attack upon the metal being washed. If the concentration of the solution is too high or too low, it attacks the aluminum and this places a serious limitation on the type of solution which may be employed.

Silicates have been used also for cleaning tin but in this case the alkalinity of the cleaning solution must be adjusted to so low a pH and the temperature of cleaner dropped to such an extent that effective cleaning can not easily be obtained. Other remedies for the corrosion of tin and aluminum by alkaline cleaners have been suggested also. In the case of tin, the use of sodium sulphite has become quite widespread in recent years. This material decreases the oxygen concentration of the cleaning solution and inhibits the corrosion of tin by alkalies. However, there is considerable corrosion after the sulphite is depleted, as it is very shortly in usual practice. Where the solution is heated in contact with air, the sodium sulphite is readily converted into sodium sulphate, which is ineffective in preventing corrosion.

Probably the most successful remedy for corrosion which has been found thus far has been the addition of chromates or dichromates to alkaline materials in the washing of soft metals. While in general these materials are quite successful in preventing corrosion, they have two serious drawbacks. They tend to coat the metal being washed with a greenish yellow film which in most cases is very undesirable. Most people are sensitive to chromates and the operators using the cleaners frequently suffer from what is known

as "chromic ulcers," which necessitate cessation of all work with material containing chromates and which require long periods of time for healing.

It is an object of the present invention to provide means by which alkaline detergents may be made safe for cleaning soft metals. The present invention has many advantages over the methods previously employed. Aluminum, tin, zinc, lead, cadmium or other soft metals or alloys thereof may be treated with solutions of extremely high pH at boiling temperatures for long periods of time without showing any evidence of corrosion. The cleaning solutions preferably have a pH of at least 10 and in many cases the pH is as high as 12 or over. The corrosion inhibitors which I employ do not decrease in effectiveness with time, as do the sulphites, but remain effective over long periods. They are without harmful effect upon the human skin and will not occasion the difficulties accompanying the use of chromates or dichromates.

I have found that the salts of mercury, either the mercurous salts or the mercuric salts, when added in proper proportion to alkalies prevent entirely the characteristic corroding effect of the alkalies on the soft metals. Although some of the mercurous salts, as for example mercurous chloride, are generally insoluble in water, they are nevertheless operative in inhibiting corrosion under the condition hereinafter described. I believe that this is due to what may be called an "auto-oxidation-reduction" reaction in which part of the mercury in the mercurous chloride is reduced to metallic mercury and the remainder is oxidized to the mercuric state, this latter portion acting as the corrosion inhibitor. Although I have not as yet definitely proved this happens, it is nevertheless a fact that mercurous chloride acts as an inhibitor in the presence of alkalies and that there is a precipitation of what appears to be metallic mercury in the solution. The mechanism whereby the corrosion is prevented is unknown but it probably can be ascribed to the formation of nonreactive protective films on the metal surfaces.

Sodium metasilicate, sesquisilicate and orthosilicate are strong alkalies, their alkalinity increasing in the order listed. It is well known that even the weakest of these, namely sodium metasilicate when used for example to wash tin or tin plate causes rapid spangling and solution of the tin even at relatively low temperature. I have found that by adding a small quantity of a mercuric salt to any of these silicates the corrosive

effect of the solution subsequently made from it is reduced to zero even at boiling temperatures over long periods of time.

The following Tables I, II and III, for example, indicate the results that have been obtained when several pieces of tin plate were heated in alkaline solutions at 60° C. for the periods of time specified. The results show the per cent loss in weight of the tin in the cases where the alkali did not contain any mercury salt and in the cases where it did contain a mercury salt as an inhibiting agent. Mercuric chloride was used in these tests as a typical mercury salt.

In Table I, the alkaline solution was a 0.5% aqueous solution of sodium metasilicate alone and also with 5% of mercuric chloride based on the weight of the sodium metasilicate.

In Table II, the alkaline solution was a 0.5% aqueous solution of trisodium orthophosphate with and without the addition of 5% of mercuric chloride based on the weight of the trisodium phosphate.

In Table III, the alkaline solution in one case was a 0.5% aqueous solution of a mixture of 40% trisodium orthophosphate and 60% sodium metasilicate. In the other case, the same solution had added to it 5% mercuric chloride based on the combined weight of the trisodium phosphate and sodium metasilicate.

Table I  
(Per cent loss in weight)

| Hours | 0.5% aqueous solution of sodium metasilicate | 0.5% aqueous solution of sodium metasilicate+5% mercuric chloride (based on weight of sodium metasilicate) |
|-------|----------------------------------------------|------------------------------------------------------------------------------------------------------------|
| 44.5  | .163                                         |                                                                                                            |
| 85.6  | .317                                         |                                                                                                            |
| 118   |                                              | 0.0                                                                                                        |
| 133.3 | .480                                         |                                                                                                            |
| 178.5 | .643                                         |                                                                                                            |
| 208.5 |                                              | 0.0                                                                                                        |
| 222.7 | .803                                         |                                                                                                            |
| 251.5 |                                              | 0.0                                                                                                        |

Table II  
(Per cent loss in weight)

| Hours | 0.5% aqueous solution of trisodium phosphate | 0.5% aqueous solution of trisodium phosphate+5% mercuric chloride (based on weight of trisodium phosphate) |
|-------|----------------------------------------------|------------------------------------------------------------------------------------------------------------|
| 49    | .194                                         | 0.0124                                                                                                     |
| 69.75 | .289                                         | 0.0147                                                                                                     |
| 90.25 | .436                                         | 0.028                                                                                                      |

Table III  
(Per cent loss in weight)

| Hours | 0.5% aqueous solution of a mixture of 40% trisodium orthophosphate and 60% sodium metasilicate | 0.5% aqueous solution of a mixture of 40% trisodium orthophosphate and 60% sodium metasilicate+5% mercuric chloride (based on weight of trisodium orthophosphate and sodium metasilicate) |
|-------|------------------------------------------------------------------------------------------------|-------------------------------------------------------------------------------------------------------------------------------------------------------------------------------------------|
| 22    | .0927                                                                                          |                                                                                                                                                                                           |
| 43    | .178                                                                                           |                                                                                                                                                                                           |
| 60.5  | .259                                                                                           |                                                                                                                                                                                           |
| 90.5  |                                                                                                | .0275                                                                                                                                                                                     |

It will be noted from Table I that where the mercury inhibiting salt was used there was no loss in weight, even after heating for over 251 hours in the sodium metasilicate solution. In the absence of the mercury salt, there was a

loss in weight of .803% after heating for 222 hours.

The mercury salts exhibit similar inhibiting effect, when they are used with trisodium orthophosphate alone as shown in Table II or with mixtures of sodium metasilicate and trisodium orthophosphate as shown in Table III.

While mercuric chloride has been referred to in the examples as a typical mercury salt which inhibits the corrosion of soft metals, I may employ other mercury salts, either mercurous or mercuric salts. The mercury salts which are effective as corrosion inhibitors according to the present invention are those which are water-soluble or which when placed in the alkaline solution to be used in cleaning the soft metal undergo a reaction which solubilizes an appreciable proportion of the mercury. These salts are referred to hereinafter as "soluble" mercury salts. I may use the soluble mercurous or mercuric salts, such as the chlorides, nitrates, acetates, salicylates or in fact any other soluble mercury salt.

Ordinarily the mercury salt should be used in an amount equal to at least 1%, based on the weight of the alkali present and generally in an amount of at least 2% by weight. When the cleaning solution is used at low temperatures, it is possible to decrease the amount of mercury salt even below the lowest figure previously given. Generally it is unnecessary to use more than 10% of the mercury salt, although more might be used without harmful effect.

The detergent solution containing the corrosion inhibitor is useful in all cases where a highly alkaline detergent is required. It may be used for example in the washing of tin plate, tubes, bakery pans, milk cans, and in tin fabricating plants. In the fabrication of tin plate, or articles made therefrom, it is often necessary to apply grease to aid in the forming operations. This may be removed by the use of a highly alkaline cleaning solution in accordance with the present invention without attack on the tin. The cleaning solutions may be used also in the treatment of aluminum. In this case also, the solution may be used to remove the grease employed in fabricating the aluminum without, however, causing alkaline corrosion of the aluminum.

For washing pans in a bakery where the pans are washed fairly frequently, so that the amount of burned on matter is not excessive, I may use a cleaning composition containing about 95% sodium metasilicate and 5% of mercuric chloride or other soluble mercury salt. This is dissolved in water to form a solution of a strength between  $\frac{1}{4}$  of 1% and 3%, generally in the neighborhood of a 1% solution. In cleaning the bakery pans, they might be boiled in the cleaning solution for an hour.

Where the deposits on the bakery pans are excessive, I might use an aqueous solution of a composition containing 95% sodium orthosilicate and 5% mercuric chloride or other soluble mercury salt and boil the pans for an hour in that solution. This provides a more alkaline solution than in the case just mentioned.

As another example, I might use a 1% aqueous solution of a composition containing 60% sodium metasilicate, 35% sodium hydroxide and 5% mercuric chloride or other soluble mercury salt where a highly alkaline solution is desired. I might add to this composition or to any of the compositions a wetting agent, such as a sodium salt of a sulfated fatty alcohol in the amount of 1-3% based on the total weight of the solids.

The soluble mercury salts also act as inhibitors of corrosion in the presence of mixtures of alkalies with soap, casein, deflocculating agents, wetting agents, abrasives and the like.

The soluble mercury salts effectively inhibit the corrosion of tin, aluminum and other soft metals by alkali-metal carbonate solutions as well as solutions of the alkali-metal phosphates and silicates. I may add sodium hydroxide or other alkali to the silicates, phosphates or carbonates in any case where it is desired to increase the alkalinity and the corrosion of the metal may be inhibited by the use of soluble mercury salts.

The invention enables the use of highly alkaline solutions in the cleaning of soft metals without corrosion of the metal. Although the invention has been described particularly in connection with preventing the corrosion of aluminum and tin, it is applicable also to the treatment of zinc, lead, cadmium or other soft metals or alloys thereof. The term "soft metal" as used here is intended to include any metal or alloy which under the proper conditions of temperature and concentration tends to be attacked or dissolved by alkaline solutions.

Although the principal use of the invention is in connection with cleaning solutions, the invention is applicable to inhibiting corrosion of alkaline compositions in general, such for example as paints or adhesives. The addition of a soluble mercury salt to an alkaline paint or adhesive will prevent the attack of the paint or adhesive on soft metals, during the time required for the paint or adhesive to set or harden.

The invention is not limited to the examples, which have been given merely for illustrative purposes, or to the preferred proportions, but may be otherwise embodied or practiced within the scope of the following claims.

I claim:

1. An alkaline detergent composition for soft metal, comprising an alkali-metal salt of the group consisting of silicate, phosphate and carbonate, said detergent composition having a pH of at least 10 in aqueous solution and which under normal conditions of use will corrode the soft metal, said detergent composition comprising at least about 1% of a mercury salt based on the weight of said alkali-metal salt to inhibit corrosion of the soft metal, said mercury salt

5 being soluble in the aqueous solution of said alkali-metal salt.

2. An alkaline detergent composition for soft metal, comprising an alkali-metal silicate, said detergent composition having a pH of at least 10 in aqueous solution and which under normal conditions of use will corrode the soft metal, said detergent composition comprising at least about 1% of a mercury salt based on the weight of said alkali-metal silicate to inhibit corrosion of the soft metal, said mercury salt being soluble in the aqueous solution of said alkali-metal silicate.

10 3. An alkaline detergent composition for soft metal, said detergent composition comprising by weight about 60 to 95% sodium metasilicate, an effective amount up to about 35% sodium hydroxide and about 1 to 10% of a mercury salt, said mercury salt being soluble in the aqueous solution of said sodium metasilicate.

15 4. An alkaline detergent composition for soft metal, said detergent composition comprising by weight about 95% sodium metasilicate and about 5% of a mercury salt, said mercury salt being soluble in the aqueous solution of said sodium metasilicate.

20 5. An alkaline detergent composition for soft metal, said detergent composition comprising by weight about 95% sodium metasilicate and about 5% mercuric chloride.

25 6. An alkaline detergent composition for soft metal, said detergent composition comprising by weight about 95% sodium orthosilicate and about 5% of a mercury salt, said mercury salt being soluble in the aqueous solution of said sodium orthosilicate.

30 7. An alkaline detergent for soft metal, said detergent composition comprising by weight about 95% sodium orthosilicate and about 5% mercuric chloride.

35 8. An alkaline detergent composition for soft metal, said detergent composition comprising by weight about 60% sodium metasilicate, about 35% sodium hydroxide and about 5% mercuric chloride.

40 9. An alkaline detergent composition for soft metal, said detergent composition comprising by weight about 60 to 95% sodium metasilicate, an effective amount up to about 35% sodium hydroxide and about 1 to 10% mercuric chloride.

CHARLES SCHWARTZ.

CERTIFICATE OF CORRECTION.

Patent No. 2,303,398.

December 1, 1942.

CHARLES SCHWARTZ.

It is hereby certified that error appears in the printed specification of the above numbered patent requiring correction as follows: Page 3, second column, line 36, claim 7, after "detergent" insert --composition--; and that the said Letters Patent should be read with this correction there-in that the same may conform to the record of the case in the Patent Office.

Signed and sealed this 19th day of January, A. D. 1943.

(Seal)

Henry Van Arsdale,

Acting Commissioner of Patents.

CERTIFICATE OF CORRECTION.

Patent No. 2,303,398.

December 1, 1942.

CHARLES SCHWARTZ.

It is hereby certified that error appears in the printed specification of the above numbered patent requiring correction as follows: Page 3, second column, line 36, claim 7, after "detergent" insert --composition--; and that the said Letters Patent should be read with this correction therein that the same may conform to the record of the case in the Patent Office.

Signed and sealed this 19th day of January, A. D. 1943.

Henry Van Arsdale,

(Seal)

Acting Commissioner of Patents.